

# UNITED STATES PATENT OFFICE.

FREDERICK M. BECKET, OF NIAGARA FALLS, NEW YORK, ASSIGNOR TO ELECTRO METALLURGICAL COMPANY, OF NEW YORK, N. Y., A CORPORATION OF WEST VIRGINIA.

## PROCESS OF TREATING TUNGSTEN ORES.

1,081,566.

Specification of Letters Patent. Patented Dec. 16, 1913.

No Drawing.

Application filed October 22, 1912. Serial No. 727,215.

To all whom it may concern:

Be it known that I, FREDERICK M. BECKET, a subject of the King of Great Britain, residing at Niagara Falls, in the county of 5 Niagara and State of New York, have invented certain new and useful Improvements in Processes of Treating Tungsten Ores, of which the following is a specification.

10 This invention relates to the treatment of such tungsten ores as contain material proportions of phosphorus, the object of the invention being the provision of methods whereby the phosphorus-content of such ores 15 may be so far reduced as to render the ores directly available for such purposes as the preparation of metals or alloys low in phosphorus. The term "ores" is herein employed to include concentrates.

20 I have found that certain ores of tungsten, including ferberite from Boulder county, Colorado, contain very considerable proportions of phosphorus, which in special cases may attain 0.6 to 0.7 per cent. Such ores 25 consist largely of iron tungstate with a gangue of silicious character, the phosphorus being usually associated both with the mineral and the gangue in extremely variable proportions. Ores presenting similar con- 30 ditions are wolframite, an iron tungstate containing considerable manganese, and hübnerite, an iron-manganese tungstate in which manganese largely predominates. Such ores are herein referred to as ores 35 of the "iron-tungstate type." I have discovered that it is possible to remove a material proportion, and in some cases all, or nearly all, of the phosphorus from these ores by a treatment involving the solution of the phosphorus in acid reagents, without substantial solution or loss of tungsten. In other words, the effect of an acid 40 treatment under proper conditions is to increase the ratio of tungsten to phosphorus,

45 expressed as  $\frac{W}{P}$ , converting high-phosphorus ores into low-phosphorus ores available for direct smelting for the preparation of low-phosphorus ferro-tungsten.

50 In the case of certain ores, a simple acid treatment of the finely-ground ore may suffice. For example, the ore, ground to suitable fineness, say 100 mesh, may be mixed with concentrated sulfuric acid (specific 55 gravity 1.84) in the approximate propor-

tions of 200 cubic centimeters of acid per kilogram of ore. The solution proceeds at ordinary room temperatures, dissolving from 30 to 90 per cent. of the phosphorus in the course of a few hours without substantial loss of tungsten, the loss of tungsten under these conditions being usually less than one per cent. At somewhat higher temperatures, say 80-100° C., the solution of phosphorus is more rapid but the loss of tungsten is materially greater. At the same time, very considerable quantities of iron are dissolved, thus effecting a concentration of the tungsten-content of the ore. Following the acid-treatment, the ore is thoroughly washed with water to remove the dissolved substances. This simple acid treatment is effective for certain ores, usually those which contain relatively small percentages of phosphorus, or

in which the ratio  $\frac{W}{P}$  is relatively high, say 250 or more. It is therefore frequently possible, by means of this acid-treatment, so to reduce the phosphorus-content of a given ore as to render it available for the direct preparation of low-phosphorus ferrotungsten. There are however many ores which do not respond to a sufficient degree to the treatment as above described, such ores being usually comparatively high in phosphorus. I have further discovered that both of the above-described classes of ore, that is to say, those which are suitable for treatment by the simple acid-solution process and those which are not suitable, may be rendered responsive to such process by suitable heat treatment, preferably by roasting under oxidizing conditions, a roast of this character being most easily and economically accomplished. For example, the ore is crushed to 10-12 mesh and subjected to an oxidizing roast, with stirring, at a red heat or somewhat lower. The acid-treatment may be applied to the roasted ores without further crushing. The efficiency of the process may however be further increased in certain cases by a finer subdivision of the ores, either before or after the roasting.

The conditions of the acid treatment as applied to the roasted ores may be substantially as above described with reference to the raw ores. Such treatment of roasted ores has been found effective to remove up to 90 per cent. or even more of the contained phosphorus, without material loss of tung-

sten. In the acid treatment of roasted ores much less iron is dissolved than in the treatment of the raw ores.

The following tabular statement gives certain illustrative results of the effects of the acid treatment alone, and of the acid treatment following an oxidizing roast:

| Sample.        | Raw ore.                               | Acid treatment only.                   | Roasting followed by acid treatment.   |
|----------------|----------------------------------------|----------------------------------------|----------------------------------------|
|                | <i>Ratio <math>\frac{W}{P}</math>.</i> | <i>Ratio <math>\frac{W}{P}</math>.</i> | <i>Ratio <math>\frac{W}{P}</math>.</i> |
| <i>a</i> ..... | 98                                     | 283                                    | .....                                  |
| <i>b</i> ..... | 146                                    | 342                                    | .....                                  |
| <i>c</i> ..... | 293                                    | 764                                    | .....                                  |
| <i>d</i> ..... | 29.8                                   | 30.3                                   | 457                                    |
| <i>e</i> ..... | 45                                     | 46.9                                   | 525                                    |
| .....          | 70.5                                   | 82.5                                   | 800                                    |

The invention is not restricted to the use of concentrated sulfuric acid as a solvent, as results of a similar character may be obtained with other acids or acid-reacting reagents, as diluted sulfuric acid, hydrochloric acid or the like. Mixed reagents may also be used, good results having been obtained with sulfuric acid containing a small proportion of nitric acid, potassium chlorate, and other oxidizing agents. Chlorin and chlorin-yielding mixtures have not proven effective for the purposes of this invention. In the use of these acid baths it may be desirable to dispose the ore in proximity to an insoluble anode connected in a direct electric circuit, for example in proximity to an anode of lead in the case of sulfuric acid, whereby the solvent effect of the acid is somewhat accentuated.

Preferably the purified ores are smelted in presence of a metallic reducing agent,

usually silicon, the reduction being accomplished in an electric furnace, in accordance with the methods disclosed in my prior patents. By this procedure it is possible to obtain a ferrotungsten which is low both in phosphorus and carbon, and which is therefore available for general use in the preparation of high grade or alloy steels or for other purposes.

I claim:

1. The process of purifying ores of the iron-tungstate type, which consists in subjecting the same to the action of a suitable acid reagent, under conditions to increase the ratio of tungsten to phosphorus.

2. The process of purifying ores of the iron-tungstate type, which consists in heating the ores, and then subjecting the same to the action of a suitable acid reagent, under conditions to increase the ratio of tungsten to phosphorus.

3. The process of purifying ores of the iron-tungstate type, which consists in subjecting the same to the action of sulfuric acid under conditions to increase the ratio of tungsten to phosphorus.

4. The process of purifying ores of the iron-tungstate type, which consists in heating the ores and then subjecting the same to the action of sulfuric acid under conditions to increase the ratio of tungsten to phosphorus.

In testimony whereof I affix my signature in presence of two witnesses.

FREDERICK M. BECKET.

Witnesses:

J. N. DEINHARDT,  
D. BURGESS.